

106/66

Patented June 20, 1933

1,915,051

32 56

## UNITED STATES PATENT OFFICE

IRA E. CRAMER, OF BEAUMONT, TEXAS, ASSIGNOR OF ONE-THIRD TO LUCIUS C.  
CRAMER, OF CONNERSVILLE, INDIANA

### BUILDING MATERIAL COMPOSITION

No Drawing.

Application filed April 10, 1930. Serial No. 443,256.

This invention relates to a new building material composition made of a concrete composed for the most part of petroleum coke and Portland cement, combined as hereinafter described; and has for its object to provide an economical and much needed building material in such districts of the United States as cannot be entered and supplied by products of the steam boiler cinder now on the market. Therefore, this invention is an effort to create the best light weight insulating building unit possible to obtain where cinders are not obtainable. Petroleum coke is generally abundant in the very districts which lack coal cinders. As a result of experiments I have discovered ways to prepare and so handle this coke as to utilize it in making a new and useful building unit which is light durable and practical in service and possesses high insulating qualities. Thus the use of this petroleum coke for building units effects the salvage of a petroleum by product now being mostly wasted, as obviously it is not in demand for fuel at the very place where oil is plentiful and more convenient to handle for burning. The product of this invention has lost the fireproof property of the cinder product, yet, on the other hand, there is gained a characteristic in this new product that not only improves but actually perfects carbon products as a material for the body part of an ideal veneer slab or block, for veneering frame residences.

To clearly describe this invention, so it may be readily understood, it is necessary to explain the essential difference between the coal cinder and this certain kind of coke, called petroleum coke. The coal cinder used in concrete is coal after it has ceased to burn, that is, after it has ceased to flame. It is coal from which the gaseous or volatile constituents have burnt, but which retains carbon capable only of further combustion without flame; in other words, it is the hard core of coal left after other parts have been burnt. But petroleum coke strictly speaking is not a cinder or ember; it is different; it has not yet been burnt; it is the dregs or final dross of the distilling process that makes gasoline, etc. While strictly speaking, it is not coal, or at

least not natural coal, yet it is more similar to coal and is used as fuel in the same manner—it is inflammable. Hence the manufacturers of cinder concrete products have not considered petroleum coke as fit material to enter their fireproof building units, and they do not employ it in their products.

Again, petroleum coke materially differs from coal cinder in another respect, i. e., it is not hard like said cinder or hard core of coal, but is comparatively soft and tender and has never, to the best of my knowledge, been utilized, as suitable material for concrete. Still another and characteristic difference is the relatively large size of the cavities or pores of petroleum coke, and it is this feature that makes it, for concrete purposes, so much superior to coal and so much different in kind from the steam boiler cinder.

It is the last two above cited characteristics of petroleum coke, i. e., its comparatively soft or tender nature and its comparatively large cavities or pores, that for building material so greatly distinguishes it from coal coke and all kinds of cinders heretofore used in the manufacture of building units. Its tenderness makes necessary a different process of using it than is used on other materials. It is the cavities or pores, above mentioned, which particularly adapt the material for use in making veneer slabs and blocks. These cavities being larger in petroleum coke, are on the average more round and pocket-shaped, often partly closed over at the surface of the lump. This allows little streams of the cement, reduced with water to a soupy or creamy state, to flow into said cavities forming roots, which dove-tail into the coke lump. These roots connected to the desired surfacing coat, (such as of sand-cement plasters, stucco, etc.), will anchor the surfacing material so it will be less likely to peel off, because where the said surfacing is applied in mold or at time of making the veneer block or slab, the above mentioned feature combined with the necessary extra portion of cement content in the aggregate qualifies this product to grip and hold such surfacing material so much more firmly than can any product of the steam boiler cinder, and such like.

70

75

80

85

90

95

100

The present invention shows that this coke can be made fit for building material; it can be semi-fire proofed, and at the same time its degree of firmness be suitably reinforced, 5 by simply leveling up to the surface the outside layer of large peculiar pores, filling them with Portland cement, (or else with a mortar made of the cement and very finely divided parts of this same coke about the size 10 of fine sand grains). This, after it sets, makes a hard casing or shell wall within the surface of the coke lump itself without submerging its farther projecting web; this 15 miniature incasing wall employs the common arch or egg-shell principle, supplies needed crushing strength to the individual lump and makes it sufficiently firm to endure mixing and molding without crushing.

This aforesaid reinforcing wall can be built 20 in said outside layer of coke pores in filling them, by either of several different modes, without departing from this invention. In one way, for instance, the larger individual lumps of coke can be spread in a single layer 25 on a wide wire cloth belt inclined and vibrated so as to gently roll the coke lumps while pouring over them a thin soupy mortar. Said mortar can be made by wetting and 30 mixing pure Portland cement or combined equal parts cement and coke, the latter finely divided into grains of the size of fine grade of ordinary masonry sand. Any process which attains this end, and fills with aforesaid material, or similar material, the peculiar 35 surface pores of said petroleum coke lumps, is comprehended by this invention. Even without this advance hardening of the larger lumps, a sufficient careful method can be employed to avoid crushing in mixing or molding, thus, without departing from this invention, the same final product may be reached. In the latter case, the portion of 40 cement, or mortar, required to fill said surface pores being added to that portion of cement required to stick each lump to the others, and hardens at the same time. And it is when employing this method of manufacture, suitable surfacing material, (sand-cement plaster or stucco, etc.), placed on the proper 45 building unit while molding it, results in an ideal veneer slab or block.

According to the present invention, concrete for my novel product is prepared by 50 mixing together the following ingredients approximately in the following proportions, and in the manner hereinafter set forth:—

Petroleum coke, three (3) parts by measure, Portland cement one (1) part by 55 measure, although these proportions can be varied from to meet conditions without departing this invention. For instance where it is desired to mold my product into very small building units, possibly as small as 60 standard size brick, it will be found more

suitable to screen out the larger lumps of petroleum coke, and to use only pieces ranging in size, from about wheat-grain size to corn-grain size, and this will require a larger proportion of cement than is required where 70 much larger building units are desired and where therefore a considerable proportion of the larger lumps of petroleum coke, (ranging from hickory nut size to egg size or larger) 75 can be included in the mixture. Also where the material is desired to stand up under heavy weight or stand severe stresses and shocks, the proportion of Portland cement can be increased accordingly, and where 80 there is not expected to be much strain or stress the proportion of petroleum coke can be accordingly increased. Therefore the proportion of petroleum coke and Portland cement may considerably differ under aforesaid 85 conditions such as the varying sized building units desired, (making convenient the use of varying proportions of larger and smaller lumps of petroleum coke) and also due to varying amount of strength 90 desired.

On one extreme, where the coke is much powdered and consists at best only of very small grains, with small building units and much strength desired, a fifty-fifty mixture 95 may be needed, i. e. equal parts by measure of the coke and cement. On the other extreme where the powdered coke is eliminated by screening it out and the smallest pieces used being about wheat-grain size, and corn-grain size, and only enough of these sizes to 100 form a filling between much larger lumps, for molding into large units, preparing for small stress or strain, one (1) part by measure of Portland cement may be found sufficient to mix with four to six (4 to 6) parts 105 of petroleum coke. And between these two extremes varying conditions will require many varying proportions of the coke and cement contents.

The preferred manner of mixing the 110 petroleum coke and Portland cement is first to dry mix them together and then mix in sufficient water to mush the mixture and to insure that the Portland cement will set hard after the mixture has been pressed into molds 115 to form building block or wall units, etc.

Anyone skilled in mixing and molding concrete can mix petroleum concrete and mold it into building units, without first experimenting, if they will observe the following 120 very simple rules, namely:—

First.—Eliminate the powder part from petroleum coke by screening it out. Also (by screening) grade the remaining coke into lump sizes to suit immediate requirements 125 and conditions.

Second.—Consider the size of grains or lumps desired to be mixed and the degree of strength desired, and for like amount of same which would require two (2) bags of 130

cement to mix it, if it were sands, gravels, or cinders of same size, use for this coke at least three (3) bags of Portland cement.

Third.—Mix this coke concrete without 5 grinding it, (as under a hoe in cases of sand and gravel concrete), or else the larger lumps will continually crush into smaller pieces and require adding more cement to maintain a given desired richness of mixture. Mix by 10 running hoe or shovel under it and turning over, or in type of cement mixer that most gently rolls it until mixed. First dry-mix it, then wet it "mush" stage; use molds adapted to wet process molding, and press it in mold 15 instead of sharp tamping it, thus avoiding crushing of larger lumps while molding.

Reinforcing agents, such as expanded metal lath, reinforcing wire or rods, metal screen cloth, etc., may if desired be incorporated or embedded in the cement-coke concrete, particularly when employed in the construction of silo walls and the like, or when molded into lintels, slabs, beams, etc., where maximum strength is desired.

25 Where a surfacing coat, such as of sand-cement plaster, stucco, etc., is applied at time of molding these building units, color material may be included in such surfacing coat without departing from this invention, yet 30 any such surfacing is not a part of this invention beyond the discovery of this particular inherent quality of petroleum coke concrete without which it would lack such extraordinary ability to grip and hold surfacing material.

Having thus described my invention what I claim as new and desire to secure by Letters Patent of the United States, is:—

1. A new material for molding into building blocks comprising the hereinafter mentioned substances in substantially the following proportions; petroleum coke lumps three parts and binder one part, said binder comprising Portland cement and petroleum coke fines.

2. A new article of manufacture, a light molded non-sweating building unit that can be nailed into and sawed, comprising lumps of petroleum oil coke providing interior and 50 exterior cells, said lumps being bound together by and having their exterior cells only filled with a mortar mixture of cement and a substantial quantity of particles of petroleum oil coke in lieu of sand.

55 In testimony whereof, I affix my signature.  
IRAE CRAMER.